

## UNITED STATES PATENT OFFICE

2,010,134

## SIZE COMPOSITION FOR ARTIFICIAL SILK

Herman S. Bosland, Paterson, N. J., and Frederick G. La Piana, Forest Hills, N. Y., assignors to Stein, Hall & Company, Inc., a corporation of New York

No Drawing. Application September 9, 1931,  
Serial No. 561,988

5 Claims. (Cl. 134—20)

This invention relates to the sizing treatment of artificial silk and rayon yarns and threads or filaments, and to improved compositions for use in carrying on such sizing treatment.

5 In the past, the weaving of fabrics from yarns and threads or filaments of artificial silks and rayon, and particularly artificial silks of the cellulose acetate type, has been attended with difficulties. The percentage of breaks in the threads 10 is excessive, and there is a tendency for the threads to become snarled. So far as we are aware, none of the sizes heretofore used with this class of textile materials has satisfactorily met these difficulties.

15 This invention relates more particularly to warp sizing of such materials, as distinguished from finish sizing. In dealing with yarns such as artificial silk yarns, which are composed of continuous fibers, different problems are met with 20 than in the treatment of yarns made up of short fibers, such as cotton and wool, or in treating yarns of real silk. In the manufacture of textile fabrics made of cotton and wool, the yarns tend to fray as they pass through the reeds and other 25 parts of the loom, due to the many loose ends, and in warp sizing such yarns, the size is primarily intended to act as a shield to prevent fraying by pasting and holding in the loose ends. On the other hand, in manufacturing textile 30 fabrics from artificial silk yarns the yarns have continuous threads and thus there is not the need for pasting loose ends down as in cotton yarns, for example. However, these continuous threads are generally somewhat weaker than cotton, wool and real silk, and have a greater tendency 35 to snap. Therefore, in the warp sizing of artificial silks, the size should operate primarily as a strengthening and lubricating element to prevent the snapping of the threads while at the same time functioning as a shield to prevent 40 fraying or snarling should a thread snap.

Furthermore, in warp sizing as ordinarily practiced, the size is to be removed from the threads after the fabric has been formed. A characteristic of artificial silk is that it is generally weaker when immersed in water or is in a wet condition and this is not true of yarns such as cotton, wool and real silk. Accordingly, artificial silk fabrics 45 cannot ordinarily be subjected to such a severe processing for the removal of a warp size as is possible with a fabric made from cotton, wool and real silk.

In weaving cellulose acetate yarns and similar 50 yarns a further difficulty is met with, namely, that such yarns are more or less water-repellent,

and consequently there is a tendency for the size to be repelled from the yarns during the sizing treatment or to adhere poorly to the yarn.

It is an object of the present invention, therefore, to provide a size having the above-mentioned strengthening and lubricating characteristics and which is also readily removable from the fabric after the formation thereof.

It is a further object of the present invention to provide a size which will readily wet and stick 10 to artificial silk yarns and threads, and when applied to the same will strengthen them and give them a smooth coating, permitting them to slip freely through the reeds and other parts of the loom with which they contact.

15 We have found that sizes which have ordinarily been used for sizing cotton and wool, such as the various starches, dextrins, natural gums, gelatin and animal glues, are unsatisfactory when it is attempted to use them for the sizing of artificial silk yarns and filaments, and particularly for warp sizing, for the reason that such sizes, either cannot be successfully applied to artificial silks due to the water-repellent character of certain of such silks or do not have the desired 20 properties of strengthening the yarns and being easily removed therefrom. We have found further that casein, and particularly certain casein-base sizes, can be successfully applied to artificial silk threads and yarns, and have all of the 25 desired characteristics above mentioned.

30 We are aware of the fact that casein in combination with various other substances has heretofore been proposed by others to be used as a finish size for cotton, wool and real silk fabrics 35 and as a coating for fabrics and paper where it is desired to make the fabric or paper waterproof, e. g., in finishing book cloth; but so far as we are aware, casein has not been used heretofore either alone or in any combination as a 40 warp size or on artificial silk fabrics. However, the problem that presents itself in the weaving of artificial silk or rayon and particularly cellulose acetate yarns, is quite different. In the first place, a warp sizing treatment of yarns and 45 threads preparatory to weaving is given for the purpose of imparting certain properties and thereby to overcome certain difficulties that are not presented in treating the finished fabric. Furthermore, certain artificial silk yarns and 50 threads and particularly those derived from cellulose acetate are more or less water-repellent and this has caused difficulties to arise in effecting a sizing of such yarns, due to the fact that there has been a tendency for the sizes hereto- 55

fore used to be repelled from the yarn during the sizing operation. On the contrary, our composition is not repelled from the yarn but wets and sticks to it, strengthening and lubricating it, and at the same time, is readily removable therefrom.

Our invention, therefore, resides in the discovery that casein alone or in combination with certain other substances is especially adapted for use in preparing a size for sizing artificial silk yarns and threads, and particularly for warp sizing thereof. While casein alone constitutes a satisfactory size under favorable circumstances, there are particular advantages in adding other substances, such as corn sugar or a similar hygroscopic material, dextrin or dextrinized starch-containing material and/or glue to the casein in forming a size for this purpose. It is also desirable, but not essential, to add a preservative such, for example, as sodium fluoride.

In the preparation of a casein size we have found that it is advantageous in certain cases to add to the casein a substantial amount of sugar or a similar hygroscopic material with or without a small amount of a preservative, such as sodium fluoride. A suitable size of this type may be prepared from a composition consisting of from about 65 to 90 parts by weight of casein, and 10 to 35 parts by weight of a suitable hygroscopic material, such as cane sugar, corn sugar or glycerine, with or without a small percentage of a suitable preservative. A specific composition which has been highly satisfactory in service consists of a mixture containing casein, sugar and sodium fluoride in about the following proportions by weight:

|                 |     |       |
|-----------------|-----|-------|
| Casein          | 70  | parts |
| Sugar           | 27½ | parts |
| Sodium fluoride | 2½  | parts |

We have discovered further that it is sometimes advantageous to add to a mixture such as above mentioned, a suitable amount of dextrin or a dextrinized starch-containing material; and in certain instances, for example, when it is desired to keep the prepared size from congealing on prolonged standing, it is advantageous to substitute glue, which may be either of animal or vegetable origin, for all or a part of the dextrinous material. A suitable size of this type may be prepared from a composition consisting of from about 50 to 80 parts by weight of casein, 40 to 10 parts of dextrin or a more or less dextrinized starch-containing material, and the balance corn or cane sugar or other suitable organic hygroscopic material. A specific example of such a composition is as follows:

|                           |    |                 |
|---------------------------|----|-----------------|
| Casein                    | 70 | parts by weight |
| Dextrinized tapioca flour | 20 | parts by weight |
| Corn sugar                | 10 | parts by weight |

The compositions of the present invention may be mixed in the dry way and then transported

to the places where they are to be used. It will be understood that the casein must be brought into a soluble form by treatment with a suitable alkaline agent, for example ammonia. This treatment may precede the mixing step or be carried out after the mixing step and conducted either in the dry way, as by contacting the casein or the dry mixture with gaseous ammonia, or by incorporating the alkaline agent into the bath used in preparing the size from the dry mixture and thoroughly disseminating such agent through the liquid mixture.

In order to prepare and apply a size from the compositions aforesaid, it is recommended, by way of example, that to about 10 pounds of composition there be added about 8 gallons of water and 7 pounds of a neutral soluble oil or other softener, for example castor oil or olive oil which has been sulphonated to a desired degree and then neutralized; a small amount of ammonia, say, 1 pint of 26 Bé. ammonia, may be added if desired. The resultant mass is then mixed and heated to about 180° F. This procedure contemplates the pretreatment of the casein or the dry mixture in the dry way with a casein solubilizing agent. In case the casein is in the insoluble form when brought into the aqueous liquid bath, its solubilization may be effected by adding a suitable quantity of aqueous ammonia and thoroughly stirring. The sizing prepared as above described is now ready for use and may be conveniently applied to the material to be treated at a temperature of about 140-160° F.

This constitutes in part a continuation of our application Serial No. 419,200, filed January 7, 1930, now Patent No. 1,914,989.

We claim:

1. A composition for use in preparing a warp size for artificial silks consisting of a preponderant proportion of casein and an organic hygroscopic material.

2. A composition for use in preparing a warp size for artificial silks consisting of a preponderant proportion of casein, a hygroscopic material, and a preservative.

3. A composition for use in preparing a warp size for artificial silks consisting of a preponderant proportion of from 65 to 90 parts by weight of casein and from 10 to 35 parts by weight of an organic hygroscopic material.

4. A composition for use in preparing a warp size for artificial silks consisting of about 70 parts by weight of casein, about 27½ parts by weight of an organic hygroscopic material, and about 2½ parts by weight of sodium fluoride.

5. A process of preparing a warp size composition for artificial silk yarns which consists in dissolving a mixture consisting of a preponderant amount of casein and a hygroscopic material in an alkaline aqueous solution.

HERMAN S. BOSLAND.  
FREDERICK G. LA PIANA.